

May 26, 1953

S. NEVIN

2,640,169

HEATED CATHODE ELECTRON MULTIPLIER

Filed June 19, 1950



Fig. 1.



Fig. 2.



Fig. 3.

INVENTOR  
SCOTT NEVIN

BY

*R.P. Morris*

ATTORNEY

## UNITED STATES PATENT OFFICE

2,640,169

## HEATED CATHODE ELECTRON MULTIPLIER

Scott Nevin, Fort Wayne, Ind., assignor to Farnsworth Research Corporation, Fort Wayne, Ind., a corporation of Indiana

Application June 19, 1950, Serial No. 169,033

6 Claims. (Cl. 313—103)

1

This invention relates to electron multiplier tubes, and more particularly to tubes of the type wherein electrons are emitted from a heated oxide coated primary emitter and strike a secondary emissive target.

In electron multiplier tubes of the type wherein secondary emission is effected by electrons from a cathode within the tube, it is desirable to use indirectly heated cathodes of the oxide coated type to obtain high initial emission in the interest of efficiency. Considerable trouble has been encountered in such tubes, in that while initially high secondary to primary emission ratios may be obtained, this ratio rapidly declines in use. It has been thought that poisoning of the secondary emissive target electrode is caused by transfer of substances from the primary cathode oxide coating to the secondary emissive layer. Consequently attempts to overcome this deficiency have been directed to a study of different oxide coatings for the cathode, and to structural designs calculated to avoid direct transfer of substances between the emitting electrodes, by evaporation or the like. Applicant has discovered that the difficulties described above can be overcome without resort to the expedients of special tube designs or cathode coating oxides. This has been accomplished by substituting tantalum as the supporting base metal for the emitting cathode oxide in place of the usual nickel base.

It is an object of this invention to provide an electron multiplier tube giving a high ratio of primary to secondary emission, stable over a long life period by providing a cathode comprising a tantalum element coated with an emissive oxide.

In accordance with a feature of this invention there is provided an electron multiplier tube comprising a primary emissive cathode, a secondary emissive electrode and a collector electrode, in which the cathode comprises a heated tantalum base coated with an electron emissive oxide.

The secondary emissive, or target, electrode may comprise known types of elements having a normally high secondary to primary electron emission ratio as for example a magnesium-silver alloy, which may be treated by an oxidizing process.

The collector electrode may consist of a wire grid, preferably a refractory metal such as tantalum. The oxide coating of the cathode may be of any known variety as for example an oxide of barium-strontium carbonate. Various forms

2

of signal control may be used such as a control grid, or other type of signal control may be supplied. The tube may be constructed with the various electrodes concentric and coaxial one with another.

The above-mentioned and other features and objects of this invention and the manner of attaining them will become more apparent and the invention itself will be best understood by reference to the following description of an embodiment of the invention taken in conjunction with the accompanying drawings, in which:

Fig. 1 illustrates a tube embodying the features of this invention;

Fig. 2 is a view of a cathode embodied in my invention partly broken away showing the features of construction, and

Fig. 3 is a set of curves illustrating typical life test measurements on tubes in accordance with the invention.

Turning to Fig. 1 there is disclosed an electron multiplier tube having an envelope 1, a cathode 2, a secondary emitting, or target, electrode 3, a control grid 4 and a collector electrode 5. Heater leads for the cathode are shown at 6, and other leads, for applying operating potentials are shown at 7, 8, 9 and 10 for the cathode, secondary emitter and collector electrode respectively. Supporting discs of mica or other suitable material are shown at 11.

The cathode 2 comprises a base metal, shown here as a sleeve 12 carrying an emitting coating 13. The coating may be any well known type of oxide, as for example an oxide of barium-strontium carbonate.

The secondary emissive electrode may for example be a silver-magnesium alloy oxidized properly to be highly emissive with respect to primary electrons impinging thereon. The collector as shown is in the form of an open cage or grid of wires which will permit the passage of high velocity electrons from the cathode to the secondary emitting electrode.

Normally the secondary emitting, or target, electrode is maintained positive with respect to the cathode, and the collector is maintained at even higher positive potential. Primary electrons emitted from cathode 2 are accelerated by the positive potential on collector electrode 5 so that most of them pass through the openings in this electrode and impinge on the target electrode 3, releasing secondary electrons. These released electrons tend to migrate to collector electrode 5 from whence they are applied over

the lead conductor 9 to a suitable output apparatus.

It is desirable to obtain a high secondary to primary electron ratio  $K$ , in the interest of efficiency. In the past with this type of tube it has been found that in many instances while  $K$  may have a fairly high value, such as 3 or more initially, this value tends to drop upon operation, and may become quite low, for example, 1.5 or so as the tube is used. In tubes of this type it has generally been the practice to use nickel as the cathode base, because it has properties which are considered desirable for indirectly heated cathodes. In making tubes with such nickel supporting sleeves it has been observed that the secondary to primary emission ratio seems generally to deteriorate rapidly in use. This indicates that in operation some deposit is made on the target electrode which poisons the surface reducing its secondary emissivity. A typical performance curve of a tube using a nickel supporting sleeve is shown at 14, in Fig. 3. It will be observed that while the  $K$  ratio is nearly 3 initially, it rapidly dropped off to the neighborhood of 2 and remained there for 350 hours of life test.

In tubes in accordance with this invention, the cathode base support is made of tantalum instead of nickel. In tubes made with such tantalum supporting sleeves, it has been observed that the  $K$  ratio builds up to an optimum value of 3 or higher and is maintained at this high value for the period of long life tests. Two typical examples of life test curves are shown at 15 and 16, Fig. 3. The tube of curve 15 started with an initial  $K$  ratio of 2.5, built up rapidly to a value of 3.25 and after 649 hours of operation still had a  $K$  ratio of 3.1. The tube of curve 16 started at a  $K$  ratio of about 3.1 built up to a ratio of 4 after 75 hours operation, and was still operating at a  $K$  ratio of 3.5 after 600 hours of operation.

Experiments were made only with tantalum in place of the nickel supports. The precise reason for the improved operation observed is not known but it is believed it may be explained on the basis of vapor pressure of the base metal. At an operating temperature of  $1100^{\circ}$  C. nickel has a vapor pressure of  $15 \times 10^{-10}$  mm. of mercury. In order to obtain a comparable vapor pressure tantalum must be heated to over  $2400^{\circ}$  C. It seems therefore that the nickel vapor may be the contaminant which poisons the secondary emitting surface. On this basis other metals of low vapor pressure might be used in place of the tantalum with comparable results. Thus, one might use tungsten or molybdenum as such supporting sleeves for the emitting oxide of the primary cathode.

Although a grid controlled multiplier has been illustrated by way of example, it should be clearly understood that the principles of the invention apply equally well to tubes wherein signal control is by other means than a grid, as by beam deflection, for example.

While I have described above the principles of my invention in connection with specific apparatus, it is to be clearly understood that this description is made only by way of example and not as a limitation to the scope of my invention.

What is claimed is:

1. An electron tube comprising, an electron tube envelope, a secondary electron emissive target electrode, a heated type primary electron emissive cathode electrode, and a collector electrode positioned within said envelope, said cathode electrode comprising a tantalum base coated with an emissive oxide.

2. An electron discharge tube according to claim 1 wherein said secondary electron emissive target electrode comprises a surface of silver-magnesium alloy and oxides of these metals.

3. An electron tube according to claim 2 wherein in said emitting oxide comprises an oxide of barium-strontium carbonate.

4. An electron multiplier tube in which the ratio of secondary emission to primary emission is maintained stable at an optimum value under operating conditions for a long life period of use of the tube, comprising a hollow cylindrical secondary emissive target electrode, an indirectly heated type primary emissive cathode comprising a tantalum sleeve coated with an emitting oxide positioned coaxially of said target electrode and a collector electrode in the form of a wire cage of tantalum mounted between said cathode and said target electrode.

5. An electron multiplier tube according to claim 4 further comprises a control grid electrode maintained between said cathode and said target electrode.

6. An electron tube according to claim 6 wherein in said emissive target electrode comprises an interior surface of magnesium silver alloy oxide.

SCOTT NEVIN.

References Cited in the file of this patent

UNITED STATES PATENTS

| Number    | Name          | Date          |
|-----------|---------------|---------------|
| 2,205,500 | Strutt et al. | June 25, 1940 |
| 2,393,803 | Nelson        | Jan. 29, 1946 |
| 2,411,601 | Spencer       | Nov. 26, 1946 |
| 2,430,218 | Eitel et al.  | Nov. 4, 1947  |
| 2,462,869 | Kather        | Mar. 1, 1949  |